

May 31, 1960

W. L. SLADE

2,938,234

METHOD FOR THE TREATMENT OF EXTRUDED POLYTETRAFLUOROETHYLENE

Filed Aug. 18, 1955



2,938,234

**METHOD FOR THE TREATMENT OF EXTRUDED POLYTETRAFLUOROETHYLENE**

Winton L. Slade, Lancaster, Pa., assignor to Raybestos-Manhattan, Inc., Manheim, Pa., a corporation of New Jersey

Filed Aug. 18, 1955, Ser. No. 529,236

5 Claims. (Cl. 18—55)

This invention relates to the treatment of extruded 15 polytetrafluoroethylene as it comes from the extruding device.

In the extrusion process, as now well understood, the polymer in powdered form is mixed with a lubricant to form a paste-like compound which can be extruded in a suitable device such as a ram-type extruder. In the preferred commercial practice, the compound is extruded vertically downward and the extrudate passes downward by gravity through a treatment apparatus comprising a relatively low temperature vaporizing zone and a relatively high temperature sinter zone. To remove the lubricant, it has been the practice to subject the extrudate in the vaporizing zone to an upwardly flowing stream of heated air which serves to vaporize and drive off the lubricant. In the sinter zone, the extrudate is subjected to a temperature sufficiently high to sinter the polymer into a homogeneous mass.

In carrying out this process, it is generally desirable to effect as complete removal of the lubricant as possible. Furthermore, the most efficient lubricants are flammable, and it has been necessary to maintain the proportion of lubricant vapor to air below the minimum explosion limit in order to prevent likelihood of fire and explosion. For these reasons, it has been necessary to control very carefully the volume and rate of flow of the air through the vaporizing zone. However, despite careful control of the air flow, the flammable lubricant sometimes catches fire.

One object of the present invention is to overcome these objections and to provide an improved process for the treatment of extruded polytetrafluoroethylene.

I have discovered that it is possible to employ a heated inert gas to effect vaporization of the lubricant, thereby eliminating the fire and explosion hazard, and eliminating the need for very careful control of the gas flow. Not only have I found that an inert gas can be efficiently employed as the lubricant-vaporizing medium but I have also found that a simple structural arrangement can be employed which will prevent any air from entering the vaporizing zone.

In the treatment of extruded polytetrafluoroethylene, it is desirable to provide a soaking zone immediately following the sinter zone to permit equalization of the temperature throughout the wall of the extrudate and to allow additional time for coalescing of the polymer. Without the use of a soaking zone it is very difficult to attain a uniform sinter temperature and to hold the extrudate at that temperature for additional time. However, in prior usages of a soaking zone employing radiant heat difficulties have been encountered in attaining the required temperature control. I have discovered that these difficulties can be overcome by the use of convection heat transfer in the soaking zone, preferably by introducing heated inert gas into this zone as well as the vaporizing zone.

A further object of this invention, therefore, is to pro-

vide an improved method in which a soaking zone is employed to best advantage and prior difficulties are overcome.

Other objects and features of the invention will be apparent from the following description with reference to the accompanying drawing, in which the single figure is a vertical sectional view of a preferred form of the apparatus employed according to this invention.

In the drawing, there is shown a hollow vertical tower 10, 1, preferably in the form of a long rigid tube or conduit of circular cross section, arranged below the extruding die 2 of an extruding device to receive the extrudate 3 as it comes from the die. The extrudate moves downwardly by gravity through the vertical treatment tower. In the course of the downward movement of the extrudate, it moves successively through the vaporizing zone 4 and the sinter zone 5. In the vaporizing zone, the lubricant is vaporized and driven off, while in the sinter zone the extrudate is subjected to heat radiated from the wall of the oven and produced by an electrical heating unit 6 which is surrounded by a thick heat-insulating jacket 7.

As thus far described, the apparatus is generally similar to that previously employed. As hereinbefore mentioned, the preferred lubricants employed in the extruding process are flammable, one such lubricant being that known as "varnish makers and painters naphtha." In the past, vaporization of the lubricant has been effected by heated air flowing upwardly through the vaporizing zone, and even though substantially pure air is employed and the proportion of lubricant vapor to air is kept well below the minimum explosion limit, fires can still occur. This comes about because some of the lubricant vapor is driven into the interior of the tubing by the heat in the vaporizing oven, and this vapor is forced by its own vapor pressure to flow down through the tubing at a rate faster than the rate of extrusion until it escapes from the open end, or if the tubing is a long continuous extrusion, until it condenses to a liquid in the cooler zones below the sinter oven. When the open end of a new extrusion first enters the sinter oven, lubricant vapor escaping from this end will usually ignite and burn like a torch. Then again, during an extrusion run, if it should happen that there are any holes in the wall of the tube, lubricant vapor escaping from these holes into the sinter oven will likewise ignite. Another possibility is that the rate of extrusion may be accidentally increased, thus releasing large quantities of lubricant vapor into the vaporizing zone in a short period of time, with the result that the minimum explosion limit is exceeded, causing fire or explosion.

In accordance with the present invention, these objections are overcome by performing all heating operations in an atmosphere of inert gas. While this gas may be introduced at the lower part of the vaporizing zone, it is preferably introduced through an entrance 8 at the lower part of the treatment tower. The inert gas may be supplied from a conventional gas generator 9. The gas flows upwardly through the sinter zone and through the vaporizing zone to an exit 10 provided at the top of the tower.

The inert gas employed may be nitrogen, carbon dioxide, superheated steam, or any gas which does not react with the lubricant vapor at the temperatures involved, or does not react exo-thermally so as to liberate large amounts of heat as in combustion. The gas may also be a mixture of inert gases. The preferred gas is a typical flue gas, or products of combustion, resulting from essentially complete burning of natural gas, or other available fuel, with approximately theoretical air. When using natural gas, the products of combustion will

be a mixture of nitrogen, carbon dioxide and water vapor, with traces of other gases but virtually no oxygen.

The inert gas is supplied at a temperature of approximately 700° to 750° F. As it passes through the vaporizing zone, its average temperature is about 400° to 500° F., and when it reaches the exit 10, its temperature is about 100° to 150° F.

For effective use of the inert gas, it is necessary to prevent air from entering the bottom of the treatment tower, and in the apparatus shown, this is accomplished by providing a water trap 11 at the bottom of the apparatus through which the extruded tubing may be passed without permitting air to enter. It is practically impossible to seal the upper end of the tower into which the soft extrudate enters, but I have found that the upper end of the tower may be left open to the air, and that this is actually advantageous. The air which enters the open end mixes with the inert gas and is drawn through the exit 10. This air has a cooling effect, with the result that the air-gas mixture drawn through the exit 10 by exhaust blower 12 has a relatively low temperature of about 100° to 150° F.

As hereinbefore indicated, the heat for sintering the polymer extrudate in the sinter zone is transferred largely or entirely by radiation from the heated walls of the oven. The use of radiant heat transfer in the sinter oven is commercially desirable because high rates of heat transfer, with corresponding allowable high rates of extrusion, are obtainable with a relatively small sinter oven occupying a small vertical height. Such a radiant-type sinter oven, while compact and efficient, is not easily controlled. Thus, it is necessary to synchronize carefully the sinter oven wall temperature with the extrusion speed, in order to avoid under-sintering or over-sintering of the polymer extrudate. The higher the sinter oven radiant temperature, the faster will be the properly synchronized extrusion speed for ideal sintering, but the more critical will be the synchronization.

Furthermore, it is desirable to provide a soaking zone immediately following the sinter zone to permit equalizing of the temperature throughout the wall of the extrudate, and to allow additional time for coalescing of the polymer, but the required temperature control in this zone is very difficult to attain if radiant heat alone is supplied.

In accordance with a further feature of the present invention, an arrangement is provided by which the use of a soaking zone is made possible and practical. As shown in the illustrated embodiment, a soaking zone 13 is provided below the sinter zone, and the inert gas is supplied at the lower part of the soaking zone so that it passes upward through that zone and then through the sinter zone and the vaporizing zone. The temperature of the inert gas is regulated at the gas generator so as to be slightly above the sintering temperature of polytetrafluoroethylene and approximately at the temperature desired in the soaking zone. As previously mentioned, the gas is preferably supplied at a temperature of approximately 700° to 750° F. The movement of the heated inert gas upward is easily attained by utilizing the chimney effect of the vertical tower. While the upwardly flowing gas, as it passes through the soaking zone and the sinter zone, is at or above the sintering temperature, the additional radiant heat from a heating unit, such as shown at 6, is ordinarily required in the sinter zone to promote rapid rise of the extrudate temperature in this zone. Some cooling of the inert gas in the vaporizing zone will ordinarily be required, and if necessary cooling of the gas at the lower part of the vaporizing zone may be effected by the use of a cooling coil 14 to which cooling water may be supplied from a source 15 by a pump 16. Such cooling of the inert gas need only be enough to prevent too rapid volatilization of the lubricant from the extrudate, a condition which may cause bubbling within the mass of the extrudate.

After the extruded tubing leaves the soaking zone 13, it is often desirable to effect a sudden, but partial cooling of the tubing through the temperature range of about 100° F. just below the transition temperature of 621° F., in order to limit the growth of crystallinity in the polymer. Apparatus for achieving this sudden, partial cooling may consist of a fine water spray, a water mist, a cold gas jet, or other means, and is shown in the illustrated embodiment as a fine water spray 17, supplied from the cooling water source 15 by pump 18, and located near the top of chamber 19.

Whether such partial cooling apparatus is used or not, the tubing descends through chamber 19 where it is required to make a turn in order to pass through the water trap, and this requires that it be maintained at a sufficiently high temperature so as to be flexible enough to make this turn. To insure sufficient flexibility of the tubing, a gas exit 20 is provided just above the water trap, so that a portion of the hot inert gas will be drawn downward through chamber 19 to the exit 20 by exhaust blower 21. This gas keeps the chamber, and the tubing within the chamber, sufficiently warm so that the tubing remains flexible enough to make the turn. Preferably, about 75% of the gas flows upwardly from the entrance 8, while 25% is drawn downward to the exit 20. Thus, in one embodiment of the apparatus, the inert gas enters through entrance 8 at the rate of 2000 cubic feet per hour, and the upwardly flowing gas is at the rate of 1500 cubic feet per hour while the downwardly drawn gas is at the rate of 500 cubic feet per hour, all gas volumes being measured under the standard conditions and on a dry basis.

The water trap shown in the illustrated embodiment is a simple means for enabling withdrawal of the tubing while excluding air. The same result can be achieved in other ways, as by providing a gasket and causing the exhaust blower 21 to draw off such air as leaks through the gasket. If desired, the tubing could be collected within the bottom chamber on a reel, and emptied batchwise at the end of a run.

Considering the over-all operation of the apparatus shown, the extrudate enters the vaporizing zone where it is exposed to heated inert gas at an average temperature of approximately 450° F., and as it passes downward through the rising heated inert gas, it loses lubricant by vaporization. It then passes into the relatively short sinter zone where it is exposed to inert gas somewhat in excess of 700° F., and it also receives radiant heat from the oven wall which may be at a temperature of about 1100° F. Principally as a result of intense radiation, it is raised quickly to approximately 700° F., during its passage through the sinter oven, but it may be unevenly heated therein. It then enters the soaking zone, still moving counter to the heated inert gas. In this zone, it receives no appreciable radiation from the wall but it is permitted to approach closely to the uniform gas temperature of about 700°, a typical desired soaking temperature, entirely by convection heat transfer. It finally passes through the cooling zone and out through the water trap.

Under no circumstances can fires or explosions result in this system, since no oxygen is present. The sintering is achieved both rapidly and uniformly and with accurate soaking. Furthermore, large volumes of inert gas are not required, as in the case of heated air where large volumes are required to maintain a proportion of air and lubricant vapor below the explosive limit. Since most of the heat used for vaporizing, and a portion of that used for sintering, comes from the combustion of fuel rather than from electrical energy, substantial operating economy is possible.

While a preferred embodiment of the invention has been described, the invention is not limited thereto but contemplates such modifications and further embodiments as may occur to those skilled in the art.

I claim:

1. A process for making tubing of polytetrafluoroethylene which comprises extruding vertically downward by means of a die a tube of a paste-like compound comprising tetrafluoroethylene polymer and a volatile, flammable lubricant, passing said tube vertically downward and sequentially through a vaporizing zone, a sintering zone, a soaking zone and a cooling zone, introducing to said soaking zone a heated inert gas at a rate of about 2000 cu. ft. per hour and at a temperature of from about the transition temperature of the polymer to about 750° F. and passing at least a portion of said heated inert gas successively through said sintering zone and said vaporizing zone, vaporizing said lubricant by means of said heated inert gas in said vaporizing zone and removing said inert gas and said vaporized lubricant from said vaporizing zone, said inert gas having an average temperature of from about 400° to about 500° F. at the point of removal from said vaporizing zone, rapidly heating said tube by means of radiant heat from a radiant surface in said sintering zone to a temperature sufficiently high to sinter said polymer, the temperature of said radiating surface being synchronized with the rate of extrusion to avoid over sintering of said polymer, maintaining said tube in said soaking zone for a time to permit equalizing of the temperature through the wall of said tube and

5

coalescing of said polymer, rapidly cooling said tube in said cooling zone to a temperature at least about 100° F. below the transition temperature of said polymer in order to limit growth of crystallinity of said polymer, and removing said tube from said cooling zone.

2. The process of claim 1 in which a portion of said heated inert gas passes from said soaking zone to said cooling zone from where it is thereafter exhausted.

3. The process of claim 1 in which said tube is cooled 10 in said cooling zone by a fine water spray.

4. The process of claim 1 wherein said heated inert gas introduced to said soaking zone is at a temperature of from about 700° to about 750° F., and the average temperature of said inert gas at the point of withdrawal 15 from said vaporizing zone is about 450° F.

5. The process of claim 4 wherein said inert gas comprises substantially oxygen-free products of combustion of a fuel.

References Cited in the file of this patent

UNITED STATES PATENTS

|           |                        |               |
|-----------|------------------------|---------------|
| 1,950,026 | Dreyfus et al. -----   | Mar. 6, 1934  |
| 1,952,877 | Mancini -----          | Mar. 27, 1934 |
| 2,232,012 | Rooney et al. -----    | Feb. 18, 1941 |
| 2,425,782 | Bludworth et al. ----- | Aug. 19, 1947 |
| 2,685,707 | Llewellyn et al. ----- | Aug. 10, 1954 |